# EUROPEAN PATENT SPECIFICATION

(11) **EP 1 563 141 B1**
(45) Date of publication and mention of the grant of the patent: **23.05.2012**
(21) Application number: 03773753.3
(22) Date of filing: 14.11.2003
(51) Int. Cl.: D21H 19/00, B05D 1/06

(54) **PROCESS FOR COATING A WEB WITH A COATING POWDER**
VERFAHREN ZUR BESCHICHTUNG EINER BAHN MITEINEM BESCHICHTUNGSPULVER
PROCEDE DE RECOUVREMENT

(30) Priority: 14.11.2002 FI 20022034
(43) Date of publication of application: 17.08.2005
(73) Proprietor: Metso Paper, Inc., 00130 Helsinki (FI)
(72) Inventor: MAIJALA, Juha, FIN-04430 Järvenpää (FI); PUTKISTO, Kaisa, FIN-33720 Tampere (FI); HAKOLA, Jyrki, FIN-04400 Järvenpää (FI); GRÖN, Johan, FIN-02360 Espoo (FI); LIPPONEN, Juha, FIN-04400 Järvenpää (FI)
(74) Representative: Hakola, Unto Tapani
(86) International application number: PCT/FI2003/000867
(87) International publication number: WO 2004/044323

(56) References cited:
- EP-A- 0 958 865
- EP-A- 0 982 120
- WO-A-02/45869
- JP-A- 3 206 200

## Description

The present invention relates to a method for coating a surface of a web, which fibrous portion consist of papermaking fibres, with a coating powder comprising steps of:
- selecting raw materials of the coating powder comprising inorganic material and polymeric binder material, the polymeric binder material having a characteristic glass transition temperature Tg above which a rubbery state plateau exists, and a dynamic modulus, which consists of a measurable elastic component G' and a measurable loss component G", so that in the rubbery state plateau the loss factor G"/G' is at the most 80% of the value, which is reached in the glass transition temperature
- forming the coating powder from the raw materials,
- allowing the web to move between electrodes, which are in different potentials,
- applying the coating powder on the surface of the web by utilizing the difference in the electric potential, and
- finishing the coated surface of the web in a process step in which the process is arranged to achieve its maximum temperature, which exceeds the glass transition temperature T_{g} of the polymeric binder material the binder being selected as defined in claim 1.

A dry surface treatment process is a known method in which dry coating powder is applied on a web. The coating powder includes inorganic material and polymeric binder material. A problem related to coating by the dry surface treatment process is a behaviour of the polymeric binder material during the process. The viscoelastic properties of polymers depend on the temperature and frequency of deformation. On the one hand, the polymeric binder material should soften and form a film at least partially in a certain process conditions because otherwise the cohesion strength of the powder-formed layer and its adhesion to the web is insufficient. On the other hand, the softened polymeric binder material must not adhere to counter surfaces with which it is in contact during the process.

The method of the invention overcomes the above-mentioned problems. It is characterized in that the polymeric binder material is selected in such a manner that when increasing the temperature above the glass transition temperature the ratio G"/G' is at the most 80% of the ratio G"/G' in the glass transition temperature.

When the ratio G"/G' is at the most 1 in the rubbery plateau the polymeric binder material does not adhere to the counter surfaces during processing. Energy and costs can be saved in the process because polymeric binder materials having a low glass transition temperature (in other words, materials having a low softening temperature) can be used. Also shorter dwell times can be used in the process.

The present invention is utilized in a dry surface treatment process in which a web is allowed to move between electrodes, which are in different potentials. The coating powder is electrically charged by at least one electrode at one side of the web, and charged particles of the coating powder are applied on the surface of the web by utilizing an electric field, which is created between the electrode at the one side of the web and at least one electrode at the other side of the web. The potential difference between the electrodes can be created by electrodes having opposite polarities, or by an electrode being either positive or negative and a ground electrode. After a coating layer has been formed on the web the coated surface of the web is finished by using heat and pressure in such a manner that the polymeric binder material at least partially melts. In the finishing step the process achieves its maximum temperature.

The preferred ranges for the thermomechanical treatment are: The temperature of 80-350°C, the linear load of 25-450 kN/m and the dwell time of 0.1-100 ms (speed 150-2500 m/min; nip length 3-1000 mm; in one passage). The thermomechanical treatment can be made by various calendering methods or calendering-like methods. The methods utilize nips formed between rolls, or substantially long nips formed between two counter surfaces. Examples of such nips are hard-nip, soft-nip, long-nip (e.g. shoe-press or belt calender), Condebelt-type calender and super-calender.

The fibrous portion of the continuous web to be treated consists of papermaking fibres. In the present application, the papermaking fibres refer to fibres obtained from trees, in other words, either fibres of a mechanical or chemical pulp or mixtures of those two.

The coating powder includes inorganic particles (e.g. ground CaCO₃ precipitated CaCO₃, kaolin, talc, TiO₂ etc.) and polymeric binder particles. Suitable polymeric materials for polymeric binder particles are for example styrene-butadiene or acrylate copolymers. The polymeric binder material may comprise several polymers, and its characteristics may be modified. The inorganic particles and the polymeric binder particles can be separate particles, or an inorganic portion and a polymeric portion may be integrated into same particles. The average diameter of the material particles is usually 0.1 - 500 µm, preferably 1 - 15 µm.

The coating powder comprises 10.1 - 99.5 wt-% (dry weight) of inorganic material and the rest is preferably polymeric binder material. The coating powder comprises preferably at least 70 wt.-% of inorganic material and more preferably at least 80 wt.-% of inorganic material. The coating powder comprises preferably at the most 99 wt.-% of inorganic material and more preferably at the most 95 wt.-% of inorganic material.

For a known polymer composition that includes an amorphous phase, there is a known or characteristic range of temperatures where the glass transition takes place. This transition region, which with increasing temperature corresponds to a change in the mechanical properties of the material, is generally described as a change from glassy to rubbery state. The glass transition temperature, which can be taken characteristic for each type of polymers, but is affected e.g. by chemical means, is usually determined in a static state. Exerting a dynamic deformation into the material shifts the transition temperature towards higher temperatures.

The viscoelastic behaviour of a material determines a flowing ability of a material. Mechanical properties of viscoelastic material under dynamic loading can be denoted by the elastic and viscous components of the dynamic modulus, which for example in torsional deformation mode are the shear storage modulus G' and shear loss modulus G".

The ratio G"/G' is called a loss factor, which typically reaches its maximum in the glass transition temperature. Above the glass transition temperature there is a range called a rubbery state plateau. In the rubbery state plateau the loss factor changes less. The loss factor in the rubbery state plateau does not exceed a level, which is at the most 80 % from the level, which is reached in the glass transition temperature. In general a level corresponding to 50 % of the glass transition temperature level is not exceeded. For polymeric binder materials, which have a distinct melting point Tₘ, the rubbery state plateau can be defined as a range between the glass transition temperature and the melting point. For materials not having a distinct melting point, the rubbery state plateau can be defined simply as a rubbery state.

The finishing step in the thermomechanical treatment causes deformations in the coating layer. The deformation properties of the whole coating are affected by e.g. the binder selection and content, additives and interactions between the binder and the pigments. When the web is not loaded (e.g. compressed) any more, some of the deformations recover and some last (permanent change). The ratio G"/G' measured for the binder indicates the formation of permanent changes within the material under deformational stresses.

The properties of the properly selected polymeric binder material during the dry surface treatment process can be described as follows: When the elastic component G' of the dynamic modulus remains stable at high enough level and the ratio G"/G' is 1 at the most in the rubbery state plateau, the adhesion of the polymeric binder material to the counter surfaces during processing is diminished. In other words, the elastic component G' shall be higher or at least equal to the loss component G" above the softening temperature of the polymeric binder material. The loss factor may be almost constant, or slightly increasing or decreasing. Preferably the loss factor is constant and maintains steady in range 0.2 - 1.0, or more preferably in range 0.2 - 0.6 when measured at elevated temperatures and conditions corresponding to the processing. The elastic modulus (the shear storage modulus) of the polymeric binder material is preferably at least 1.0 x 10⁵ Pa when measured at fixed conditions corresponding the thermomechanical treatment. This high elasticity typically requires polymer crosslinking to a some degree. Hence, the polymeric binder material is selected in such manner that when increasing the temperature above the glass transition temperature the ratio G"/G' is at the most 80% of the ratio G"/G' in the glass transition temperature. The glass transition temperature is determined in the same conditions as the loss factor. The ratio G"/G' is at the most 1 in the rubbery state plateau between the glass transition temperature of the polymeric binder material and the maximum processing temperature (the temperature in the coating material).

The viscoelastic properties during a thermomechanical treatment can be determined according to ASTM D5279-01 in a following manner: An even film of 1 to 3 mm in thickness is manufactured from a polymeric binder material. The film is put under torsional stress, and at the same time the film is allowed to move through a specific temperature range. As the viscoelastic properties vary between measuring conditions, it is important to specify the conditions in each case. The used temperature range was -30 - 130°C and the temperature rise 3°C/min. The used frequency was 1 Hz. The torsional loading created shearing in the material with an adjusted strain of 16 % (in relation to a full circle).

In the following, the invention is explained by referring to figures in which
- Figures 1 and 2: show curves representing an elastic modulus and a loss factor as a function of temperature.

In figure 1, the elastic component G' of the shear modulus is represented by a curve A, and the loss factor G"/G' is represented by a curve B. The curves show properties of a polymeric binder material, which has acceptable characteristics for use in the dry surface treatment process. The elastic modulus is at least 1,0 x 10⁵ Pa, and the loss factor is at the most 1. The characteristic glass transition temperature of the material is 24°C (measured in the static state). However, a peak in the curve B representing the glass transition temperature has been shifted towards higher temperatures due to a dynamic measurement method.

In figure 2, the elastic component G' of the shear modulus is represented by a curve C, and the loss factor G"/G' is represented by a curve D. The curves show properties of a polymeric binder material, which has no acceptable characteristics for use in the dry surface treatment process. The elastic modulus is below 1,0 x 10⁵ Pa when the temperature exceeds 75°C, and the loss factor is over 1 when the temperature exceeds 110°C. The characteristic glass transition temperature of the material is 24°C. It is very probable that this polymeric binder material disadvantageously sticks onto surfaces during processing.

The invention is not restricted to embodiments explained above but it may vary in the scope of the claims.

## Claims

1. A method for coating a surface of a web, which fibrous portion consist of papermaking fibres, with a coating powder comprising steps of:
- selecting raw materials of the coating powder comprising inorganic material and polymeric binder material, the polymeric binder material having a characteristic glass transition temperature Tg above which a rubbery state plateau exists, and a dynamic modulus, which consists of a measurable elastic component G' and a measurable loss component G", so that in the rubbery state plateau, the loss factor G"/G' is at the most 80 % of the value, which is reached in the glass transition temperature (the viscoelastic properties being determined according to ASTM D5279-01, conditions as defined herein),
- forming the coating powder from the raw materials,
- allowing the web to move between electrodes, which are in different potentials,
- applying the coating powder on the surface of the web by utilizing the difference in the electric potential, and
- finishing the coated surface of the web in a finishing process step in which the process is arranged to achieve the maximum process temperature, which exceeds the glass transition temperature T_{g} of the polymeric binder material,
**characterized in that** the polymeric binder material is selected in such a manner that the ratio G"/G' is at the most 1 in the rubbery state plateau between the glass transition temperature and the maximum process temperature..

2. The method according to claim 1, **characterized in that** the elastic component G' is at least 1.0 x 10⁵ Pa in a temperature range, which is below the maximum process temperature.

3. The method according to claim 1 or 2, **characterized in that** the loss factor in the rubbery state plateau is at the most 50 % of the value, which is reached in the glass transition temperature.

4. The method according to claim 2, **characterized in that** the polymeric binder material is crosslinked.

5. The method according to any of the claims 1 to 4 , **characterized in that** the ratio G"/G' is constant and maintains steady in range 0.2 - 0.6.

## Patentansprüche

1. Verfahren zum Beschichten mittels Beschichtungspulver einer Oberfläche einer Bahn, deren fasriger Anteil aus Fasern zur Papierherstellung besteht, aufweisend folgende Schritte:
- Auswählen von Rohmaterialen des Beschichtungspulvers aufweisend anorganisches Material und polymerisches Binde-Material, wobei das polymerische Binde-Material eine charakteristische Vitrifizierungstemperatur Tg, oberhalb der ein gummielastisches Zustands-Plateau vorliegt, sowie ein Dynamik-Modul hat, das aus einer messbaren elastischen Komponente G' und einer messbaren Verlustkomponente G" besteht, sodass der Verlustfaktor G"/G' auf dem gummiartigen Zustands-Plateau maximal 80 % des Wertes beträgt, der bei der Vitrifizierungstemperatur erreicht wird (die viskoelastischen Eigenschaften werden gemäß ASTM D5279-01 bestimmt, Zustandsbedingungen wie hierin definiert),
- Bildung des Beschichtungspulvers aus den Rohmaterialen,
- Schaffung der Möglichkeit, die Bahn zwischen Elektroden laufen zu lassen, die unterschiedliche Potenziale aufweisen,
- Aufbringen des Beschichtungspulvers auf die Oberfläche der Bahn unter Anwendung der Differenz in dem elektrischen Potenzial, und
- Fertigstellung der beschichteten Oberfläche der Bahn in einem Endbearbeitungsschritt, bei dem der Prozess dazu bestimmt ist, die maximale Prozesstemperatur zu erreichen, die die Vitrifizierungstemperatur Tg des polymerischen Binde-Materials übersteigt,
**dadurch gekennzeichnet, dass** das polymerische Binde-Material derart ausgewählt wird, dass das Verhältnis G"/G' am gummielastischen Zustands-Plateau zwischen der Vitrifizierungstemperatur und der maximalen ProzessTemperatur maximal 1 ist.

2. Verfahren nach Anspruch 1, **dadurch gekennzeichnet, dass** die elastische Komponente G' mindestens 1,0 x 10⁵ Pa in einem Temperaturbereich beträgt, der unterhalb der maximalen Prozesstemperatur liegt.

3. Verfahren nach Anspruch 1 oder 2, **dadurch gekennzeichnet, dass** der Verlustfaktor beim gummielastischen Zustands-Plateau maximal 50% des Wertes beträgt, der bei der Vitrifizierungstemperatur erreicht wird.

4. Verfahren nach Anspruch 2, **dadurch gekennzeichnet, dass** das polymerische Binde-Material quervernetzt ist.

5. Verfahren nach einem der Ansprüche 1 - 4, **dadurch gekennzeichnet, dass** das Verhältnis G"/G' konstant ist und beständig in dem Bereich 0,2 - 0,6 verbleibt.

## Revendications

1. Procédé pour revêtir une surface d'une bande, dont la partie fibreuse consiste en fibres de fabrication du papier, avec une poudre de revêtement comprenant les étapes de :
- sélectionner des matières premières de la poudre de revêtement comprenant une matière inorganique et une matière liante polymère, la matière liante polymère ayant une température de transition vitreuse Tg caractéristique au-dessus de laquelle existe un plateau d'état caoutchouteux, et un module dynamique, qui consiste en une composante élastique mesurable G' et une composante de perte mesurable G", de sorte que, dans le plateau d'état caoutchouteux, le facteur de perte G"/G' est au plus 80 % de la valeur qui est atteinte dans la température de transition vitreuse, les propriétés viscoélastiques étant déterminées selon ASTM D5279-01, conditions telles que définies ici,
- former la poudre de revêtement à partir des matières premières,
- permettre à la bande de se déplacer entre des électrodes qui sont à des potentiels différents,
- appliquer la poudre de revêtement sur la surface de la bande en utilisant la différence dans le potentiel électrique, et
- finir la surface revêtue de la bande dans une étape de traitement de finition dans laquelle le traitement est agencé pour obtenir la température de traitement maximale, qui dépasse la température de transition vitreuse Tg de la matière liante polymère,
**caractérisé en ce que** la matière liante polymère est choisie de telle manière que le rapport G"/G' est au plus 1 dans le plateau d'état caoutchouteux entre la température de transition vitreuse et la température de traitement maximale.

2. Procédé selon la revendication 1, **caractérisé en ce que** la composante élastique G' est au moins 1,0 x 10⁵ Pa dans une plage de température qui est inférieure à la température de traitement maximale.

3. Procédé selon la revendication 1 ou 2, **caractérisé en ce que** le facteur de perte dans le plateau d'état caoutchouteux est au plus 50 % de la valeur qui est atteinte dans la température de transition vitreuse.

4. Procédé selon la revendication 2, **caractérisé en ce que** la matière liante polymère est réticulée.

5. Procédé selon l'une quelconque des revendications 1 à 4, **caractérisé en ce que** le rapport G"/G' est constant et se maintient stable dans une plage de 0,2-0,6.
